

# UNITED STATES PATENT OFFICE.

WILLIAM A. McADAMS, OF BAY SHORE, NEW YORK.

## ALUMINUM ALLOY AND METHOD OF PRODUCING THE SAME.

1,076,137.

Specification of Letters Patent.

Patented Oct. 21, 1913.

No Drawing.

Application filed March 20, 1912. Serial No. 685,035.

*To all whom it may concern:*

Be it known that I, WILLIAM A. McADAMS, a citizen of the United States, and resident of Bay Shore, in the county of Suffolk and State of New York, have invented a new and useful Improvement in Aluminum Alloys and Methods of Producing the Same, of which the following is a specification.

My invention consists in an aluminum alloy and in the method of producing the same, said alloy comprising a novel combination of materials in novel proportions, producing a composition of matter especially well adapted for casting, said composition being very strong and resonant and having a permanent superior luster.

The alloy is composed of aluminum, zinc, silver and copper combined in substantially the following proportions by weight; aluminum sixty parts, zinc twenty parts, silver sixteen and one-half parts, and copper five parts.

In producing the alloy, the method which I have found to be the best is as follows: The aluminum is melted and raised to a sufficiently high temperature to cause it to show a red color. The copper is then introduced into the aluminum and afterward the silver is added. The temperature of the mass is then lowered until it shows substantially no red color. The zinc is then introduced and the mass agitated thoroughly when it will be ready for casting.

The alloy composed of the above materials and combined in proportions substantially as above set forth, will present a beautiful

permanent luster of a superior quality. It will be very resonant and will have great strength for so light a composition.

What I claim is:

1. An aluminum alloy composed of aluminum, zinc, silver and copper, the proportion by weight of aluminum being greater than that of the zinc, the proportion of zinc by weight being greater than that of the silver and the proportion by weight of the silver being greater than that of the copper.

2. An aluminum alloy composed of aluminum, zinc, silver and copper combined in substantially the following proportions by weight: aluminum sixty parts, zinc twenty parts, silver sixteen and one-half parts and copper five parts.

3. The method of forming an aluminum alloy composed of aluminum, zinc, silver and copper, consisting in melting the aluminum and raising to a temperature sufficiently high to cause it to show a red color, then introducing the copper and the silver, then lowering the temperature of the mass until it shows substantially no red color and then introducing the zinc and thoroughly agitating the mass.

In testimony, that I claim the foregoing as my invention, I have signed my name in presence of two witnesses, this 18th day of March, 1912.

WILLIAM A. McADAMS.

Witnesses:

F. GEORGE BARRY,  
C. S. SUNDGREN.

Copies of this patent may be obtained for five cents each, by addressing the "Commissioner of Patents, Washington, D. C."